

J. F. MONNOT.  
SHIP PLATE AND HULL.  
APPLICATION FILED NOV. 27, 1907.

1,060,930.

Patented May 6, 1913.



Attest:

  
Frank E. Rappman

by

Inventor:  
John F. Monnot  
Marble, Mitchell & Rappman  
Atty's

# UNITED STATES PATENT OFFICE.

JOHN FERREOL MONNOT, OF NEW YORK, N. Y., ASSIGNOR TO DUPLEX METALS COMPANY, OF NEW YORK, N. Y., A CORPORATION OF NEW YORK.

## SHIP PLATE AND HULL.

1,060,930.

Specification of Letters Patent.

Patented May 6, 1913.

Application filed November 27, 1907. Serial No. 404,154.

*To all whom it may concern:*

Be it known that I, JOHN F. MONNOT, a citizen of the United States, residing at New York, in the county of New York and State of New York, have invented certain new and useful Improvements in Ship Plates and Hulls; and I do hereby declare the following to be a full, clear, and exact description of the same, such as will enable others skilled in the art to which it appertains to make and use the same.

My invention relates to improvements in ship plates and ship hulls, and comprises a ferrous metal plate weld-coated on its exposed face, and preferably weld-coated on all faces and edges, with a less oxidizable metal such as copper; and also comprises a hull having plates and rivets of such clad metals.

It is well known that iron or steel plates of ship hulls are extremely subject to corrosion or rusting and that the paint with which such plates are usually covered offers only partial protection against such corrosion. Furthermore, it is well known that submerged steel plates are in many cases extremely apt to accumulate barnacles, seaweed and other marine growths, materially affecting the speed of the vessel. For the protection against the latter trouble, hulls are sometimes coppered; that is, covered with sheet copper, brass, Muntz's metal, tobin bronze, and similar cupriferous metals, but to avoid galvanic action between the steel hull plates and such coatings, it is necessary to interpose intermediate sheathings of wood, or like material, which, however, is only partially successful in protecting against such corrosion.

The speed of a vessel, of course, is affected largely by the skin friction produced by its wetted surface. This is one of the reasons for using the smooth copper sheathings. Steel is not a homogeneous metal, being com-

posed of fibers or crystals of various different compounds of carbon and the element iron, together, generally, with more or less comparatively pure iron. Separated graphitoidal carbon is also a common constituent.

A polished surface of steel or iron shows polished exposed faces of these different bodies and under the common laws of electro-chemistry they form galvanic couples which much promote corrosion when such a polished surface is immersed in a reactive

fluid such as seawater. This corrosion is, however, localized, one spot forming a positive element and dissolving, and another, a negative element, which remains comparatively uncorroded. The corroded spots form pits or depressions as compared with the uncorroded spots, thereby on the one hand much increasing skin friction and on the other giving opportunity for barnacles and marine growths to cling. There is also trouble from corrosion where brass or bronze circulating pipes, sea water connections and the like, terminate in the skin of the vessel.

The clad plates herein described, may be produced from clad metal ingots produced as described in my Patent No. 853,716, dated May 14, 1907, and in various of my pending applications including particularly applications Sr. Nos. 391,673 filed September 6, 1907 and 400,843 filed November 5, 1907, whereby ingots of steel weld-coated with copper, brass, and other relatively non-oxidizable metals, may be produced. In ingots and in sheets, rods and the like, produced from such ingots, the coating so applied is weld-united to the steel or other base, being inseparable therefrom by the action of stripping tools, such as cold chisels, and by temperature changes or shock, and the union between the coating and the base metal being apparently stronger than the coating metal itself. In rolling or extending such ingots into sheets, and the like, the coating is drawn out substantially in the same proportion as is the base metal, without rupture or the development of pores or flaws, the coating being, even when extremely thin, absolutely impervious to liquids and having all the desirable qualities of metal solidified from the molten state. The coating is further very hard as compared with ordinary copper, brass, etc., owing to the support it receives from the underlying stronger steel weld-united to it, and presents to the action of water, a smooth planished surface entirely homogeneous and therefore free from the conditions which produce local galvanic couples in steel plates as before referred to. The copper in the co-extension of the two metals being compressed between the relatively stiff steel on the one side and the working tools on the other while held against lateral yielding by the existence of a basal weld union assumes throughout its mass a peculiar hard texture similar to the

surface texture of hard drawn wire, all porosities being obviated and the copper being made very dense, hard and compact. The metal being coated in the ingot and drawn down from the ingot to sheets and the like, the coating may be very thin while preserving all the desirable qualities of the coating metal.

Heretofore it has been proposed to coat steel plates with copper and other metals by casting molten copper against the plates. Such coatings being applied to the plates themselves, the coating itself must be quite thick, and therefore adds materially to the cost and weight of the plates, while adding practically not at all to the strength. I have found that if copper be cast against steel at ordinary casting temperatures, no union results, the coating so formed being at most adherent and not coherent to the steel; while if the coating metal so cast be at a very much higher temperature and be maintained in contact with the steel at such temperature for any material length of time, it will dissolve much of the steel and will in turn be greatly impaired in quality by the dissolved iron, the alloy produced being extremely brittle, coarse and full of blow holes, bubbles and the like. In fact, under such conditions both of the metals become what is technically known as "rotten." There is also apt to be between the metals a seam, spot or surface of non-union into which sea water may penetrate, producing to an enhanced degree, the very local action which it is the object of the coating to avoid. This will not only lead to destructive corrosion of the steel but will lead eventually to peeling off or exfoliation of the coating.

The accompanying drawings show a portion of a ship hull, comprising plates such as above described, also a portion of such a plate.

In said drawings: Figure 1 shows an elevation of a plurality of ship plates and a frame member connected together; Fig. 2 shows a transverse section through such plates and frame member on the line 2-2 of Fig. 1; Fig. 3 shows a similar section on the line 3-3 of Fig. 1; and Fig. 4 shows two plates and a strap connected together by rivets and also composed of compound metal such as before referred to.

In the said drawings, 5, 5, designate the plates, the vertical edges of which abut one against the other and the horizontal edges of which are over-lapped in the usual manner, and 6 designates a frame member.

7, 7 designate strap plates, and 8, 8 rivets uniting the plates 5 and said straps. Each of these plates, and preferably the rivets themselves, are composed of clad steel such as before referred to, for example, copper clad steel, the copper being weld-united, to render it inseparable from the steel, by the

method hereinbefore referred to. In the drawings, 9 designates the base of strong metal such as steel, and 10 the coating of relatively non-oxidizable metal, such as copper. It is preferable that the plates shall be coated on both sides and also on the edges and in the rivet holes with the coating metal 10, and since it is impracticable to coat the plates themselves after they are rolled down to size or nearly so, I draw the coating metal over the edges and into the rivet holes so as to completely cover such edges and the sides of the rivet holes, in the process of cutting the plates to size and of punching the rivet holes. This I may do by the method and means described in my applications Sr. No. 293,410 filed December 26, 1905, and Sr. No. 303,916 filed March 2, 1906, comprising in brief the use of blunt-edged tools which sever the metal by an obtunding action as distinguished from a strict cutting action, such tools being able to draw the coating metal over the severed edges of the core or base metal, substantially as indicated in Fig. 4. The frame members 6 may also be composed of clad metals, such as before referred to, although in general this is not necessary, it being usually practicable to protect the inner surfaces of the skin of the vessel, by paint, cement, and the like, so that corrosion will not take place, even under the influence of bilge water.

In some cases vessel hulls have been plated with plates of aluminum or aluminum alloys, and it has been found that the aluminum or aluminum alloy is subject to corrosive or solvent action on the part of sea water, which has resulted in material eating away of the plates, the latter being greatly weakened and rendered spongy. Where, for extreme lightness or other reasons, plating with aluminum is desired, these aluminum or aluminum alloy plates may be weld-coated, in the ingot, with copper or other metal not subject to this corrosive action, and thereby all the advantages heretofore stated with reference to the clad steel plates, are obtained.

Where it is desired to close the joints between the plates against the entrance of sea water, by means other than the usual paint, this may be done by running molten solder or brazing brass into the joints. In Fig. 4, 11 indicates such a filling.

What I claim is:—

1. A ship plate comprising a core or base of one metal weld-coated with a less corrodible cupriferous metal, said metals having been co-extended and said cupriferous metal having throughout its mass a hard, dense and compact structure.

2. A ship plate comprising a core or base of one metal weld-coated on both sides with a less corrodible cupriferous metal, said metals having been co-extended and said

cupriferous metal having throughout its mass a hard, dense and compact structure.

3. A ship plate comprising a core or base of one metal weld-coated on its exposed face 5 and on its edges with a less corrodible cupriferous metal, said metals having been co-extended and said cupriferous metal having throughout its mass a hard, dense and compact structure.

10 4. A ship plate comprising a core or base of steel weld-coated with cupriferous metal, the united metals having been co-extended and said cupriferous metal having throughout its mass a hard, dense and compact structure.

15 5. A ship plate comprising a core or base of steel weld-coated on both sides with cupriferous metal, the united metals having been co-extended and said cupriferous metal 20 having throughout its mass a hard, dense and compact structure.

6. A ship plate comprising a core or base of steel weld-coated on its exposed face and on its edges with cupriferous metal, the united metals having been co-extended and 25 said cupriferous metal having throughout its mass a hard, dense and compact structure.

7. A ship's plate consisting on one side of a steel plate and on the other side of a dense and homogeneous plate of cast copper, the 30 surface of demarcation between said plates being sharply defined, but the respective metals interpenetrating to such extent as to secure perfect union of the plates, substantially as described.

In testimony whereof I affix my signature, 35 in the presence of two witnesses.

JOHN FERREOL MONNOT.

Witnesses:

K. P. McELROY,  
H. M. MARBLE.